

## UNITED STATES PATENT OFFICE

2,261,047

## LUBRICANT

Peter A. Asseff, Cleveland, Ohio, assignor to The Lubri-Zol Corporation, Wickliffe, Ohio, a corporation of Ohio

No Drawing. Application July 28, 1941,  
Serial No. 404,361

14 Claims. (Cl. 252—35)

This invention relates as indicated to improved lubricants and more particularly to compounded lubricants which comprise a mineral lubricating oil base, the properties of which affecting its use as a lubricant will be improved by the inclusion therein of an addition agent.

Refined mineral lubricating oils while useful over a wide range of applications, are, nevertheless, not satisfactory for certain uses either on account of their tendency to deteriorate or on account of their inability to withstand high film pressures or otherwise perform the lubricating function required.

It is a principal object of this invention, therefore, to provide a compounded lubricant which while including a mineral oil base has properties which cannot be secured by the use of mineral oil alone.

Other objects of the invention will appear as the description proceeds.

To the accomplishment of the foregoing and related ends, said invention then comprises the features hereinafter fully described and particularly pointed out in the claims, the following description setting forth in detail certain illustrative embodiments of the invention, these being indicative, however, of but a few of the various ways in which the principal of the invention may be employed.

Broadly stated, the compounded lubricating composition of this invention may be defined as comprising a major amount of a hydrocarbon oil, such as mineral lubricating oil, and a minor amount of a zinc salt of an acidic reaction product obtained by reacting phosphorus pentasulphide with a cyclo-aliphatic alcohol.

In the foregoing broad statement of this invention the addition agent has been defined in terms of its mode of preparation and desirably and necessarily so on account of the difficulty in a more precise identification of the molecule characterizing the addition agent. As a matter of fact the addition agent is probably a mixture of different constituents and it is for this reason that the same is best defined, as above indicated, in terms of its mode of preparation. The addition agent may be prepared as indicated by reacting phosphorus pentasulphide with a cyclo-aliphatic alcohol in the preparation of an intermediate acidic reaction product and the zinc salt then prepared of such acidic reaction product.

Alternatively, the final product may be prepared in a single step or in concurrent steps by reacting together phosphorus pentasulphide the alcohol, and zinc oxide. In this case, it is prob-

able that the reaction which forms the intermediate acidic reaction product, and the reaction of such acidic reaction product with zinc oxide to form the final salt, take place simultaneously.

The following is a list of cycloaliphatic alcohols which may be used in carrying out this reaction, and in such list, the specific examples are arranged substantially in the order of preference.

- 10 Methyl cyclohexanol
- Ethyl cyclohexanol
- Propyl cyclohexanol
- Amyl cyclohexanol
- Sterols, e. g. "Cosmol" (a cyclic alcohol derived from wool-fat)
- Cyclohexanol
- Methyl cycloheptanol
- Methyl cyclopentanol
- Cycloheptanol
- 20 Cyclopentanol

It is not necessary that the cycloaliphatic alcohol used for this purpose be a pure compound. It may consist of a mixture of cycloaliphatic alcohols and such mixtures are often particularly advantageous. An example of such material is the mixture of alcohols resulting from the hydrogenation of commercial cresol. The "methyl cyclohexanol" referred to hereafter is the product thus obtained. A mixture of alkylated cyclohexanols consisting principally of ethyl and propyl cyclohexanols has also been found particularly suitable for this purpose.

The cycloaliphatic alcohols which contain the cyclohexane nucleus, for example cyclohexanol and the alkylated cyclohexanols, are particularly useful cycloaliphatic alcohols for my purpose because they are commercially available and produce a product which has advantageous properties.

40 Of the cycloaliphatic alcohols in general those are preferred which have a total of less than ten carbon atoms. The alkylated cycloaliphatic alcohols are particularly suitable. In this case, it is best to have the alkyl group contain less than six and preferably less than four carbon atoms.

Since a specific example of the addition agents of the present invention which has been found of especial utility is the zinc salt of the acidic reaction product obtained by reacting phosphorus pentasulphide with methyl cyclohexanol, the details of the manufacture of such material will be given as illustrative of the mode of manufacture of the similar addition agents comprised within the broad statement of the invention,

This process may be divided into two parts, i. e.

- (a) The preparation of the acid ester, and
- (b) The preparation of the metallic salt of such acid ester.

(a) PREPARATION OF THE ACID ESTER

Five moles of methyl cyclohexanol and one mole of  $P_2S_5$  were mixed with an amount of benzene equal in volume to the amount of cyclohexanol and placed in a flask equipped with a reflux condenser, a thermometer and a mechanical stir. The flask was placed in a water bath at approximately  $100^{\circ} C.$  and refluxed for four hours. The batch was then cooled to about  $60^{\circ} C.$  and washed once with an equal volume of water at  $60^{\circ} C.$  The benzene was removed from the wash material by distillation at atmospheric pressure. A typical batch in the preparation of the acid ester in the mode above defined was as follows:

|                                               |            |
|-----------------------------------------------|------------|
| Wt. of methyl cyclohexanol                    | grams      |
| Moles of methyl cyclohexanol                  | -----      |
| Weight of $P_2S_5$                            | grams      |
| Moles of $P_2S_5$                             | -----      |
| C. c. of benzol used as solvent               | -----      |
| C. c. of $60^\circ C.$ $H_2O$ used in washing | -----      |
| Weight of product                             | grams      |
| Temp. of reaction, $^\circ C$ :               |            |
| Bath temp                                     | $^\circ C$ |
| Vapor temp                                    | $^\circ C$ |
| Time of reaction                              | hours      |

It is believed that the reaction between phosphorus pentasulphide and the alcohol produces a mixture of compounds of the type represented by acid thiophosphate esters. For example:



where:

R is the cyclo-aliphatic radicle derived from the alcohol.

R' is hydrogen or R.

The final product, if this assumption is correct, would then consist of the salts derived from the acid ester by replacing the replaceable hydrogen of such esters with zinc.

(b) PREPARATION OF THE METALLIC SALT

### *First method.*

The acid ester resulting from step (a) above was mixed with enough water to make a 15-20% mixture. This solution was made neutral to phenolphthalein with 30% aqueous caustic. The acid was neutralized at 80-90° C. To the soda-salt solution was added an aqueous solution of zinc chloride. The reaction mixture was stirred at 80-90° C. for fifteen minutes, and then allowed to settle. The time required for the separation of the water from the salt was about fifteen minutes. The water was then poured off and the zinc salt dissolved in twice its volume of benzene. The water and benzene were removed by vacuum distillation at about seven inches vacuum. The maximum temperature of

distillation was 100° C. A typical batch in the preparation of the zinc salt of the reaction product of phosphorus pentasulphide and methyl cyclohexanol was as follows:

|    |                                                        |            |
|----|--------------------------------------------------------|------------|
| 5  | Grams of salt obtained                                 | 980        |
|    | Per cent yield                                         | 89.5       |
|    | Time of reaction between NaOH and acid                 | minutes 15 |
| 10 | Time of reaction between Na salt and ZnCl <sub>2</sub> | minutes 15 |
|    | Temperature of reaction, °C:                           |            |
|    | NaOH+acid                                              | 80-90      |
|    | Na salt+ZnCl <sub>2</sub>                              | 80-90      |
| 15 | C. c. of benzol used for dehydration                   | 2000       |
|    | Temperature of dehydration                             |            |
|    | °C maximum                                             | 100        |

### Hydration

| Second method |                          | Grams |
|---------------|--------------------------|-------|
| 20            | Methyl cyclohexanol      | 865   |
|               | Phosphorus pentasulphide | 333   |
|               | Zinc oxide               | 100   |

The methyl cyclohexanol and zinc oxide are placed in a container and heated to 180° F. Then the phosphorus pentasulphide is added in finely divided form so that it will pass a 40 mesh screen. The phosphorus pentasulphide is added over a period of about 40 minutes so that the temperature does not exceed 212° F. The temperature is then raised to 320° F. over a period of one hour and maintained at that temperature for an additional one-half hour. The yield of product is 1167 grams, and may be:

- 35 (a) dissolved in an equal weight of mineral oil and filtered hot after the addition of 2% by weight of a filter aid such as Filtral; or  
(b) dissolved in an equal weight of benzol, filtered, and the benzol removed by evaporation under vacuum.

### *Third method.*

The materials and the amounts are the same in this method as in the second method. The methyl cyclohexanol and phosphorus pentasulphide are mixed in a flask and maintained at a temperature of 212° F. by means of a water bath for seven hours. The zinc oxide is then added, and the temperatures raised over a period of one hour to 320° F., and maintained at that temperature for one hour. The yield is 1170 grams, and the final solution and purification may be the same as for the second method.

#### *Fourth method*

|                          | Pounds |
|--------------------------|--------|
| Methyl cyclohexanol      | 2975   |
| Phosphorus pentasulphide | 1137.5 |
| Zinc oxide               | 391    |

60 The methyl cyclohexanol and phosphorus pentasulphide are heated to 210° F., and the temperature is maintained there for five and one-half hours. The pressure is then reduced to give a vacuum equivalent to five inches of mercury, 65 absolute pressure, for one-half hour to remove the unreacted alcohol, hydrogen sulphide, etc. The mixture is cooled to 140° F. and zinc oxide added. The temperature is maintained at 140° F. for three hours. A vacuum equivalent to three 70 inches of mercury, absolute pressure, is applied and the temperature raised to 210° F., and that temperature maintained for nine hours. Three thousand pounds of a neutral oil are added together with 2% of filter aid, and the solution is 75 filtered at a temperature of about 200° F. The

yield of product, exclusive of the oil, is 3800 pounds.

Specific examples of addition agents contemplated for use in this invention are given in Table A below with an indication of the percentages of the various elements found therein by actual analysis.

TABLE A

| Example No. | Salt of the reaction product of— | And—                                | Sulphur | Phosphorus | Metal 10 |
|-------------|----------------------------------|-------------------------------------|---------|------------|----------|
|             |                                  |                                     | Percent | Percent    | Percent  |
| a.....      | Zinc methyl cyclohexanol.        | P <sub>2</sub> S <sub>3</sub> ..... | 14.6    | 7.7        | 7.5      |
| b.....      | Zinc amyl cyclohexanol.          | P <sub>2</sub> S <sub>3</sub> ..... | 14.0    | 7.5        | 8.5 15   |
| c.....      | Zinc cosmol.                     | P <sub>2</sub> S <sub>3</sub> ..... | 9.82    | 4.11       | 4.36     |
| d.....      | Zinc borneol.                    | P <sub>2</sub> S <sub>3</sub> ..... | 11.0    | 5.96       | 6.40     |
| e.....      | Zinc cyclohexanol.               | P <sub>2</sub> S <sub>3</sub> ..... | 19.3    | 8.95       | 8.17     |

Representative examples of lubricating compositions of the present invention were tested 20 by means of a 2½ H. P. single-cylinder, liquid-cooled, four cycle gasoline engine, rated at 1800

the lubricant tested, its comparison with an untreated base oil both as to physical properties and performance in the engine tests.

TABLE B

| Example | Composition                                                                                               |
|---------|-----------------------------------------------------------------------------------------------------------|
| 1       | Untreated SAE 30 naphthenic motor oil having a V. I. of 5.                                                |
| 2       | Example 1+1% zinc salt of the reaction product of P <sub>2</sub> S <sub>3</sub> with methyl cyclohexanol. |
| 3       | Example 1+1% zinc salt of the reaction product of P <sub>2</sub> S <sub>3</sub> with amyl cyclohexanol.   |
| 4       | Example 1+2% zinc salt of the reaction product of P <sub>2</sub> S <sub>3</sub> with amyl cyclohexanol.   |
| 5       | Untreated SAE 30 solvent refined Mid-Continent motor oil having a V. I. of 96.                            |
| 6       | Example 5+1% zinc salt of the reaction product of P <sub>2</sub> S <sub>3</sub> with methyl cyclohexanol. |
| 7       | Example 5+2% zinc salt of the reaction product of P <sub>2</sub> S <sub>3</sub> with methyl cyclohexanol. |
| 8       | Example 5+2% zinc salt of the reaction product of P <sub>2</sub> S <sub>3</sub> with borneol.             |
| 9       | Untreated conventionally refined SAE 20 Pennsylvania motor oil having a V. I. of 103.                     |
| 10      | Example 9+1% zinc salt of the reaction product of P <sub>2</sub> S <sub>3</sub> with methyl cyclohexanol. |
| 11      | Example 9+2% zinc salt of the reaction product of P <sub>2</sub> S <sub>3</sub> with methyl cyclohexanol. |

TABLE C

|                                        | 1     | 2    | 3  | 4    | 5    | 6    | 7    | 8    | 9    | 10   | 11   |
|----------------------------------------|-------|------|----|------|------|------|------|------|------|------|------|
| Engine tests at—                       |       |      |    |      |      |      |      |      |      |      |      |
| 30 hours:                              |       |      |    |      |      |      |      |      |      |      |      |
| Piston rating.....                     | D     | B    | A- | A    | D    | B+   | A    | B-   | D    | A-   | B+   |
| Number of rings stuck.....             | 0     | 0    | 0  | 0    | 0    | 0    | 0    | 0    | 0    | 0    | 0    |
| Percent filling of oil ring slots..... | 30    | 0    | 0  | 0    | 0    | 0    | 0    | 0    | 25   | 0    | 0    |
| Bearing loss in mgs.....               | 12    | 6    | 10 | 32   | 25   | 16   | 5    | 15   | 8    | 7    | 13   |
| 60 hours:                              |       |      |    |      |      |      |      |      |      |      |      |
| Piston rating.....                     | D     | C-   | B+ | A    | D    | B    | A-   | C+   | D    | B+   | B    |
| Number of rings stuck.....             | 1     | 0    | 0  | 0    | 0    | 0    | 0    | 0    | 2    | 0    | 0    |
| Percent filling of oil ring slots..... | 90    | 5    | 0  | 0    | 0    | 0    | 0    | 0    | 85   | 0    | 0    |
| Bearing loss in mgs.....               | 60    | 12   | 15 | 52   | 60   | 24   | 10   | 14   | 13   | 12   | 23   |
| 90 hours:                              |       |      |    |      |      |      |      |      |      |      |      |
| Piston rating.....                     |       | O    | A- | D    | B-   | B+   | C-   |      |      | B-   | B+   |
| Number of rings stuck.....             |       | 0    | 0  | 1    | 0    | 0    | 0    | 0    |      | 0    | 0    |
| Percent filling of oil ring slots..... |       | 10   | 0  | 0    | 0    | 0    | 0    | 0    |      | 0    | 0    |
| Bearing loss in mgs.....               |       | 19   | 63 | 107  | 31   | 14   | 16   |      |      | 17   | 30   |
| 120 hours:                             |       |      |    |      |      |      |      |      |      |      |      |
| Piston rating.....                     |       |      | A- |      | B    | A-   | C-   |      |      | C    | B    |
| Number of rings stuck.....             |       |      | 0  |      | 0    | 0    | 0    |      |      | 0    | 0    |
| Percent filling of oil ring slots..... |       |      | 0  |      | 0    | 0    | 0    |      |      | 5    | 5    |
| Bearing loss in mgs.....               |       |      | 67 |      | 37   | 20   | 24   |      |      | 22   | 38   |
| 150 hours:                             |       |      |    |      |      |      |      |      |      |      |      |
| Piston rating.....                     |       |      | A- |      | B-   | B+   | C    |      |      | B    |      |
| Number of rings stuck.....             |       |      | 0  |      | 0    | 0    | 0    |      |      | 0    |      |
| Percent filling of oil ring slots..... |       |      | 0  |      | 0    | 0    | 5    |      |      | 5    |      |
| Bearing loss in mgs.....               |       |      | 73 |      | 36   | 22   | 27   |      |      | 33   |      |
| Drain analysis:                        |       |      |    |      |      |      |      |      |      |      |      |
| Percent vis. increase.....             | 79.0  | 52.6 |    | 74.5 | 30.2 | 26.5 | 28.2 | 42.0 | 31.8 | 56.9 | 57.5 |
| Cont. carbon residue.....              | 2.40  | .91  |    | 1.81 | 1.43 | .73  | 1.06 | 1.13 | 1.39 | 1.84 | 2.27 |
| Naphtha insoluble.....                 | 15.90 | 33.2 |    | 27.6 | 1.2  | 9.2  | 1.6  | 4.2  | 3.5  | 1.4  | 8.6  |
| Acid number.....                       | .38   | .25  |    | .54  | 1.93 | .22  | .37  | .52  | .28  | .26  | .64  |
| Almen film strength.....               | 4     | 8    |    | 4    | 10   | 11   |      |      | 4    | 6    | 9    |

R. P. M. The procedure used was as follows:

The engine was loaded by means of a fantype 50 brake which applied a load of 1½ H. P. at 1600

R. P. M. The engine was run for ten minutes at 1200 R. P. M. and then the speed was increased to 1600 R. P. M. The following conditions were maintained constant during the remainder of the test—

Coolant temperature ..... °F. 345  
Oil temperature ..... °F. 225

Air fuel ratio ..... 12.7:1

The engine was stopped at 30 hour periods for inspection of piston, piston skirt, piston rings, connecting rod bearings, etc. The engine was equipped with removable connecting-rod bearings consisting of lead-bronze with a steel backing. These bearings were weighed at the beginning of the test and at each 30 hour inspection period. Before each new test, the engine was thoroughly cleaned and equipped with new piston, piston rings and with new connecting rod bearings.

In the following Table B will be found a tabulation of several lubricating compositions of the present invention and in following Table C will be found a tabulation of the characteristics of 75

The zinc salts produced in accordance with the several modes outlined hereinbefore are all new compositions of matter and are being claimed as such.

One of the principal uses of these zinc salts is in lubricating compositions for the purposes previously explained, and, in the manufacture of a finished composition for use as a lubricant in the crank cases of internal combustion engines, the oil base will be preferably a highly-refined mineral lubricating oil. The range of viscosity for such oil may be from about 100 to about 1000 seconds Saybolt Universal at 100° F. or from about 20 to about 100 seconds Saybolt Universal at 210° F. The preferred range of viscosities for the oil base are from about 150 to about 750 seconds Saybolt Universal at 100° F. or from about 40 to about 75 seconds Saybolt Universal at 210° F.

For certain uses the oil base will be preferably a high V. I. oil. Generally for such uses the oil base should have a V. I. of at least 50 and preferably at least 85 (Dean and Davis System).

The concentration of the zinc salt in the finished lubricant will be largely determined by the particular use for which the composition is designed and the particular characteristics of the

base oil or base composition to which they are added. In general, in compounded lubricating oils useful in Diesel engines, the concentration of these zinc salts will range from about .1% to about 4%, and preferably from .5% to 2.5%.

One of the particular uses of the zinc salts of my invention is in lubricating compositions which also contain so-called "detergents," particularly of the metal-containing type. Among the detergents with which these zinc salts may be used in combination are the metal phenates, and especially the alkaline earth metal phenates.

Although the addition agents contemplated hereby have a certain degree of detergent action, particularly in certain types of oils, when used as the sole addition agent, highly advantageous results may be obtained by using these addition agents with others, notably other oil-soluble organic metal compounds which, themselves, effect a higher degree of detergency when used in hydrocarbon oils. Examples of such organic metal compounds are the oil-soluble salts of:

Organic acids produced by oxidation of petroleum fractions  
Naphthenic acids  
Fatty acids  
Halogenated fatty acids, such as dichlor stearic acid  
Aromatic acids such as phenyl stearic acid and chlorophenyl stearic acid  
30 Sulphonic acids, e. g. sulphonic acids derived from petroleum  
Substituted phosphorus acids containing an organic substituent, e. g. the aliphatic, cyclo-aliphatic, and aromatic acid esters of phosphoric acid, thio phosphoric acids, phosphorous acid and thio phosphorous acids

The oil-soluble metallic phenates may also be used, such as those derived from such phenolic compounds as:

Alkylated phenols such as cetyl phenol and lauryl phenol  
Esters of salicylic acid such as lauryl salicylate and cetyl salicylate  
45 Halogenated alkyl phenols and esters of phenolic acids such as lauryl chlorophenols and lauryl chlorsalicylate  
Sulphides and polysulphides derived from phenol and alkylated phenols, such as di(tertiary amyl hydroxy-phenyl) sulphides di(tertiary amyl hydroxy-phenyl) disulphides

Specific examples of such detergent addition agents are the following:

Calcium naphthenate  
Cobalt naphthenate  
Aluminum naphthenate  
Aluminum chlorophenyl stearate  
Aluminum cetyl phenate  
Calcium oleate  
Calcium dichlor stearate  
Cobalt dichlor stearate  
Calcium phenyl stearate  
Calcium chlorophenyl stearate  
Calcium cetyl phenate  
Calcium lauryl phenate  
Magnesium phenate of lauryl salicylate  
Calcium lauryl chlorophenate  
70 Magnesium phenate of lauryl chlorsalicylate  
Calcium phenate of di(tertiary amyl hydroxy-phenyl) sulphide  
Calcium salt of mono-cetyl phosphate  
Calcium salt of di-cetyl phosphate

5 Calcium salt of di-lauryl phosphate  
Aluminum salt of mono-cetyl phosphate  
Aluminum salt of di-cetyl phosphate  
Calcium salt of mahogany acids (petroleum sulphonates)

10 Barium salt of mahogany acids  
Sodium salt of mahogany acids  
Chromium salt of mahogany acids  
Cobalt salt of mahogany acids

The zinc salts of this invention may advantageously be used with detergents comprising combinations of oil-soluble metallic compounds. Examples of such combinations are:

- 15 (a) The combination of a metallic phenate with a metallic salt of a substituted phosphorus acid containing an organic substituent.  
(b) The combination of an oil-soluble metallic alcoholate with an oil-soluble metallic salt of a substituted phosphorus acid containing an organic substituent.  
(c) The combination of an oil-soluble metallic phenate with an oil-soluble metallic salt of a sulphonic acid.  
(d) The combination of an oil-soluble metallic alcoholate with an oil-soluble metallic salt of a sulphonic acid.

Specific examples of combinations of this type are:

EXAMPLE I

|                                | Per cent |
|--------------------------------|----------|
| Calcium cetyl phenate          | .5       |
| Calcium cetyl phosphate        | .25      |
| 35 Zinc salt of this invention | .5       |
| Mineral lubricating oil        | Balance  |

EXAMPLE II

|                             | Per cent |
|-----------------------------|----------|
| Calcium cetyl phenate       | .5       |
| Calcium cetyl phosphate     | .5       |
| Zinc salt of this invention | .75      |
| Mineral lubricating oil     | Balance  |

EXAMPLE III

|                             | Per cent |
|-----------------------------|----------|
| Aluminum butoxide           | .1       |
| Calcium cetyl phosphate     | .75      |
| Zinc salt of this invention | .75      |
| Mineral lubricating oil     | Balance  |

EXAMPLE IV

|                                                                                                                              | Per cent |
|------------------------------------------------------------------------------------------------------------------------------|----------|
| Calcium salt of mahogany acids (sulphonic acid produced by the treatment of a petroleum fraction with fuming sulphuric acid) | 1.2      |
| Calcium salt derived from the alkylated phenol sulphide disclosed in U. S. Patent No. 2,139,766                              | .8       |
| 60 Zinc salt of this invention                                                                                               | .5       |
| Mineral lubricating oil                                                                                                      | Balance  |

EXAMPLE V

|                                                                              | Per cent |
|------------------------------------------------------------------------------|----------|
| Calcium salt of mahogany acids                                               | 1.2      |
| 65 Calcium salt of the condensation product of formaldehyde with amyl phenyl | .5       |
| Zinc salt of this invention                                                  | .75      |
| Mineral lubricating oil                                                      | Balance  |

EXAMPLE VI

|                                | Per cent |
|--------------------------------|----------|
| Calcium salt of mahogany acids | 1.2      |
| Aluminum butoxide              | .1       |
| Zinc salt of this invention    | .75      |
| 75 Mineral lubricating oil     | Balance  |

## EXAMPLE VII

|                                                                                                             | Per cent   |
|-------------------------------------------------------------------------------------------------------------|------------|
| Calcium salt of an acid produced by the oxidation of a fraction of a solvent-refined paraffinic mineral oil | .7         |
| Calcium salt derived from the alkylated phenol sulphide disclosed in U. S. Patent No. 2,139,766             | .15        |
| Zinc salt of this invention                                                                                 | .5         |
| Mineral lubricating oil                                                                                     | Balance 10 |

The foregoing specific examples, it will be observed, are in each instance lubricating compositions in which the mineral oil contains the zinc salt of this invention in combination with two other components. These have been given as representative not only of such three-component compositions, but also of two-component compositions which may be produced by the omission, from any of the above-named specific examples, of either one or the other of the two addition agents with which the zinc salt is shown in combination.

Additional specific examples of combinations in which the zinc salt is used with only one other detergent are as follows:

## EXAMPLE VIII

|                             | Per cent |
|-----------------------------|----------|
| Calcium cetyl phenate       | .5       |
| Zinc salt of this invention | .5       |
| Mineral lubricating oil     | Balance  |

## EXAMPLE IX

|                                | Per cent |
|--------------------------------|----------|
| Calcium salt of mahogany acids | 1.6      |
| Zinc salt of this invention    | .75      |
| Mineral lubricating oil        | Balance  |

## EXAMPLE X

|                                                  | Per cent |
|--------------------------------------------------|----------|
| Magnesium phenate derived from lauryl salicylate | .75      |
| Zinc salt of this invention                      | 2.00     |
| Mineral lubricating oil                          | Balance  |

## EXAMPLE XI

|                             | Per cent |
|-----------------------------|----------|
| Calcium phenyl stearate     | 1.00     |
| Zinc salt of this invention | 1.00     |
| Mineral lubricating oil     | Balance  |

## EXAMPLE XII

|                             | Per cent |
|-----------------------------|----------|
| Cobalt chlorphenyl stearate | .5       |
| Zinc salt of this invention | .75      |
| Mineral lubricating oil     | Balance  |

It will be noted that the addition agents of this invention contain, in a single compound, the combination of a cycloaliphatic radicle, a thiophosphate radicle, and the element, zinc. It has been discovered that this combination of constituents produces a material having a particularly desirable combination of properties for use in lubricating oil to be used in the crank cases of internal combustion engines under conditions of severe service. This combination of properties includes the following:

- (1) High solubility in oils of high viscosity index;
- (2) Detergent action or resistance to sludge-forming tendencies; and
- (3) Controlled sulphur activity, contributing corrosion-inhibiting properties and resistance to the formation of acidic materials during oxidation.
- (4) Ability to increase film strength of the oil.

In the past, it has not been found possible to 75

compound addition agents which would reduce corrosive tendencies, and the tendency to produce acidic materials during oxidation, without increasing the tendency to form deleterious deposits. By the use of the addition agents of this invention, however, the corrosive tendency and the formation of acidic materials are reduced while, at the same time, reducing the tendency to form harmful deposits.

Other modes of applying the principle of the invention may be employed, change being made as regards the details described, provided the features stated in any of the following claims or the equivalent of such be employed.

I, therefore, particularly point out and distinctly claim as my invention:

1. A lubricating composition comprising a major amount of a hydrocarbon oil and a minor amount of the zinc salt of an acidic reaction product obtained by reacting phosphorus pentasulfide with an alkylated cyclohexanol in which substantially all of the alkyl groups have less than six carbon atoms.

2. A lubricating composition comprising a major amount of a hydrocarbon oil and a minor amount of the zinc salt of an acidic reaction product obtained by reacting phosphorus pentasulfide with an alkylated cyclohexanol in which substantially all of the alkyl groups have less than four carbon atoms.

3. A lubricating composition comprising a major amount of mineral lubricating oil and a minor amount of the zinc salt of an acidic reaction product obtained by reacting phosphorus pentasulfide with a methyl-cyclohexanol.

4. A lubricating composition comprising a major amount of mineral lubricating oil and a minor amount of the zinc salt of an acidic reaction product obtained by reacting phosphorus pentasulfide with an amyl-cyclohexanol.

5. A lubricating composition comprising a major amount of mineral lubricating oil and from about .1% to about 4% of the zinc salt of the reaction product obtained by reacting one mole of phosphorus pentasulfide with approximately five moles of methyl-cyclohexanol.

6. A lubricating composition comprising a major proportion of mineral lubricating oil and from about .1% to about 4% of the zinc salt of di(methylcyclohexyl) dithiophosphate.

7. A composition of matter for use as an addition agent in lubricants comprising an oil base and the zinc salt of an acidic reaction product obtained by reacting phosphorus pentasulfide with a methyl-cyclohexanol.

8. A corrosion-inhibiting composition comprising an oil vehicle and in solution therein an effective amount of a product obtained by reacting together zinc oxide, methyl cyclohexanol and phosphorus pentasulfide.

9. A lubricating composition comprising a major proportion of lubricating oil suitable for use in the crank cases of internal combustion engines, with the properties of such composition affecting its use as a lubricant under conditions of extreme stress such as are encountered in Diesel engines and the like, and having its resistance to deterioration and the formation of acidic and varnish forming constituents improved by incorporating

70 therein from about 0.5% to about 2.5% based on the amount of lubricating oil of a zinc salt of an acidic reaction product obtained by reacting phosphorus pentasulfide with an alkylated cyclohexanol in which substantially all of the alkyl groups have less than six carbon atoms.

10. A lubricating composition comprising a major amount of mineral lubricating oil and a minor amount of the zinc salt of an acidic reaction product obtained by reacting phosphorus pentasulfide with a propyl-cyclohexanol.

11. A lubricating composition comprising a major amount of mineral lubricating oil and from about .1% to about 4% of the zinc salt of the reaction product obtained by reacting one mole of phosphorus pentasulfide with approximately five moles of an alkylated cyclohexanol in which substantially all of the alkyl groups have less than six carbon atoms.

12. A lubricating composition comprising a major proportion of mineral lubricating oil and from about .1% to about 4% of the zinc salt of a di(alkylcyclohexyl)dithiophosphate in which

substantially all of the alkyl groups have less than six carbon atoms.

13. A composition of matter for use as an addition agent in lubricants comprising an oil base and the zinc salt of an acidic reaction product obtained by reacting phosphorus pentasulfide with an alkylated cyclohexanol in which substantially all of the alkyl groups have less than six carbon atoms.

14. A corrosion-inhibiting composition comprising an oil vehicle and in solution therein an effective amount of a product obtained by reacting together zinc oxide, phosphorus pentasulfide and an alkylated cyclohexanol in which substantially all of the alkyl groups have less than six carbon atoms.

PETER A. ASSEFF.